

N. E. SIBLEY.

FLESH FILE.

APPLICATION FILED JAN. 7, 1916.

1,203,918.

Patented Nov. 7, 1916.



FIG. 1.

FIG. 2.

FIG. 3.

WITNESS

A. C. Fairbanks,

INVENTOR.

Nettie E. Sibley,

BY

Frank A. Cutten,

ATTORNEY.

# UNITED STATES PATENT OFFICE.

NETTIE E. SIBLEY, OF SPRINGFIELD, MASSACHUSETTS.

## FILESH-FILE.

1,203,918.

Specification of Letters Patent.

Patented Nov. 7, 1916.

Original application filed November 8, 1913, Serial No. 799,912. Divided and this application filed January 7, 1916. Serial No. 70,757.

*To all whom it may concern:*

Be it known that I, NETTIE E. SIBLEY, a citizen of the United States of America, residing at Springfield, in the county of 5 Hampden and State of Massachusetts, have invented a new and useful Flesh-File, of which the following is a specification, the same being a divisional part of my application filed in the United States Patent Office 10 November 8, 1913, and serially numbered 799,912.

My invention relates to improvements in abrading devices or implements for removing calluses, excrescences such as hard corns, 15 and other unnatural or undesirable thickened and hardened flesh formations from the feet and other parts of the body, and said invention resides in the peculiar combination of parts and elements which enter 20 into the construction of the file, and in the process for making the composition employed in the construction thereof, all as hereinafter set forth.

The object of my invention is to produce 25 a practical and economical implement of the class described above, which not only possesses the necessary abrading qualifications made available by convenient means, but is antiseptic so that there is no danger of injurious effects of any kind following the 30 application of the implement or file to the flesh, even though such file came in contact with the blood through broken tissue. It is needless to say that this antiseptic feature 35 is of the utmost importance in an implement which is brought so intimately into relation with the flesh of the human body.

Crushed quartz is the best and practically 40 the only suitable abrading material known for application to the flesh or cuticle. Owing to the peculiar nature of such material it is difficult, if not impractical or impossible, to unite and apply it in the form 45 of a coating of proper thickness on a body member of wood, and to secure it in such form to such member, as must be done in the construction of my file, wherefore it becomes necessary to use for this purpose a compound of paste and glue, neither paste 50 nor glue alone being adequate for such purpose.

Attention is further called to the fact that much difficulty exists in the matter of selecting antiseptics of sufficient potency, antiseptics which at the same time have no injurious effect on the cuticle or in case they 55 reach the blood, and which can be properly and advantageously combined with crushed quartz, a difficulty that I have in and by this invention entirely overcome. 60

Other objects and advantages will appear in the course of the following description.

I attain the objects and secure the advantages of my invention in part by the means 65 illustrated in the accompanying drawings, in which—

Figure 1 is a side elevation of a file which is a practical embodiment of my invention; Fig. 2, an edge elevation of said file, and, 70 Fig. 3, a central transverse longitudinal section through the same.

Similar numerals refer to similar parts throughout the several views.

As clearly shown in the drawings, the file 75 in the physical aspect of its complete form consists of a flat body portion made preferably of wood and divided into a handle 1 and a blade or shank 2, and a coating 3 of abrading antiseptic materials held together 80 and caused firmly to adhere to said shank by means of a compound of paste and glue. The shape of the shank 2 and that of the handle 1 may vary to a greater or less extent, but said shank should have substantially 85 parallel sides, or, in other words, should be generally flat in order that the coating 3 may be applied thereto to the best advantage. The coating 3 covers both sides and edges and the point or forward end of the 90 shank 2, so that said shank is completely incased in said coating and the shank portion of the complete file is at all points available for abrading purposes.

The coating 3 consists of powdered quartz, 95 boric acid, borax, oil of sweet birch, and thymol. These materials or ingredients are combined in substantially the following proportions:—To 100 pounds of the quartz are added one and one-half pints of the acid and 100 one ounce of borax, and one-half ounce of the oil and one ounce of thymol. The boric

acid and borax are added to the quartz and with the hands thoroughly mixed therewith. The oil of sweet birch is dissolved in three ounces of alcohol, then the thymol is added, 5 and this solution is sprayed over the quartz and also mixed thoroughly therewith as in the other case. The mixture thus prepared is sifted before using, if necessary. As a binder and affixer for the above mixture, I 10 employ flour paste and ground glue combined while hot. The shank 2 is dipped into the adhesive mixture or glue-paste, and then what may be termed the quartz mixture is poured over the already coated surface of 15 said shank with the result that the latter mixture is formed into and forms finally the coating 3 which is hard and permanent except as worn away by use. Two dippings and two applications of the quartz mixture, 20 usually about two days apart, are required to form the coating 3.

The abrading and antiseptic mixture or compound is prepared by first thoroughly commingling with a quantity of powdered 25 quartz proportionately small quantities of boric acid and borax, and then spraying thereon and thoroughly mixing therewith a proportionately small quantity of oil of sweet birch dissolved in alcohol and having

added thereto a proportionately small quantity of thymol. 30

What I claim as my invention and desire to secure by Letters Patent, is—

1. The process of making an abrading and antiseptic mixture or compound, for flesh 35 files, consisting in mixing with powdered quartz boric acid and borax, in spraying such mixture with oil of birch dissolved in alcohol and to which thymol has been added, and in mixing all of the said elements together. 40

2. An abrading and antiseptic coating, for flesh files, consisting of a quantity of powdered quartz having thoroughly worked into it proportionately small quantities of boric 45 acid and borax, a proportionately small quantity of oil of sweet birch dissolved in alcohol and having added thereto a proportionately small quantity of thymol, said oil and thymol also being thoroughly worked 50 into said quartz with said acid and borax, and a binder of paste and glue for the aforesaid elements.

NETTIE E. SIBLEY.

Witnesses:

F. A. CUTTER,  
A. C. FAIRBANKS.